

(No Model.)

A. DE LODYGUINE.  
ILLUMINANT FOR INCANDESCENT LAMPS.

No. 575,668.

Patented Jan. 19, 1897.

*Fig. 1.*



*Fig. 2.*



WITNESSES:

George H. Winslow.  
D. C. Teeter

INVENTOR  
Alexander de Lodyguine  
BY  
Jerry and Mackay  
ATTORNEYS.

# UNITED STATES PATENT OFFICE.

ALEXANDER DE LODYGUINE, OF PITTSBURG, PENNSYLVANIA.

## ILLUMINANT FOR INCANDESCENT LAMPS.

SPECIFICATION forming part of Letters Patent No. 575,668, dated January 19, 1897.

Application filed April 10, 1894. Serial No. 507,010. (No specimens.)

*To all whom it may concern:*

Be it known that I, ALEXANDER DE LODYGUINE, a citizen of Russia, residing at Pittsburgh, in the county of Allegheny and State of Pennsylvania, have invented a new and useful Improvement in Illuminants for Incandescent Lamps and Methods of Making Same, (Case No. 569,) of which the following is a specification.

10 My invention relates to improvements in incandescent electric lamps, and more particularly to lamps of the type set forth in my pending application, Serial No. 457,227, filed January 4, 1893, wherein an all-metal illuminant is employed.

15 In the above-named application I have described a generic process for the manufacture of illuminants for incandescent lamps whereby the incandescing material is deposited 20 upon a central fillet, which latter serves as a temporary support in manufacture, and not as a translating device for converting electric into actinic energy. In said application I have further described a specific series of 25 steps whereby metallic chromium may be deposited upon a fillet in the form of an illuminant.

30 The invention herein set forth is generically identical with that disclosed and claimed in the above-named application, but is specifically distinct therefrom in that it relates to a 35 method or process whereby an illuminant may be produced by the deposit upon a fillet of a metal, one or more of whose gaseous chlorin compounds may be safely mixed with hydrogen, and upon application of heat to the mixture will be deposited in metallic form therefrom.

40 My present invention also includes the illuminant for incandescent lamps composed of such a metal, and the metals which I have hitherto found best adapted for use in this process in the manufacture of this product are molybdenum and tungsten.

45 In the accompanying drawings, Figure 1 is a median section of an incandescent lamp containing my invention, and Fig. 2 is a section of the portion *x x* and *y y* of an illuminant made in accordance with my invention 50 and showing the fillet within the same.

Although I have shown in the drawings this illuminant as used in a stopper-lamp, it will be understood that my invention relates to a

particular method for making illuminants and to a particular form of illuminant, irrespective of the kind of lamp wherein it is used. 55

As set forth in my above-named application, my invention contemplates the use of a conducting-fillet of a nature capable of resisting heat and of supporting, at least temporarily, the metal of the illuminant without entering into chemical combination therewith. For this purpose I prefer a very fine platinum wire, the diameter of which shall be small with relation to the outside diameter of the 65 illuminant to be formed thereon. In practice I have found a platinum fillet .001 of an inch in diameter to be suitable, although I have found it desirable to use even finer fillets in order to secure a higher resistance and a shorter 70 illuminant for a given candle-power.

It will of course be understood that the dimensions above given for the fillet are only examples of those which may be used. The length and diameter of the fillet will of course 75 depend upon the candle-power, watts per candle-power, and life of the lamp which it is desired to make. Upon this fillet a metal of high resistance and of a very refractory nature is deposited, and the process of deposition is continued until the proper size of illuminant is produced. Upon passing a proper current through the resulting structure a bright and lasting light is produced. So far the process herein described is identical with that set forth in my above-named application. In said application I set forth, among other things, that it was possible to use molybdenum and tungsten as illuminants by depositing them in this manner, and I further outlined two specific treatments whereby 80 this might be accomplished. My present invention relates to one of these treatments and contemplates the use of any highly-refractory metals whose gaseous chlorin compounds, 85 upon mixture with hydrogen, deposit themselves in metallic form upon a heated surface. The two metals named above belong to this 90 category.

In depositing metals having the above-named chemical properties the following treatment is employed, and although the chlorids or chlorates of these metals may be used as the gaseous compound from which upon mixture with hydrogen the metals may be 100 deposited, I have found that the oxychlorids

of molybdenum and tungsten possess advantages for use in this treatment which render them peculiarly valuable in this connection. While, therefore, leaving it to be distinctly understood that my invention contemplates the use of chlorids, chlorates, or any other gaseous chlorin compounds of those metals which upon mixture with hydrogen deposit the metals themselves upon a heated surface, I shall proceed to describe my process in this case as carried out when the oxychlorids are used. In this branch of my process the oxychlorid is volatilized by heat and is brought into contact with the fillet in the presence of a stream of hydrogen. The fillet is heated by the passage of an electric current and the metallic oxychlorid being reduced by the hydrogen deposits the pure metal upon the surface of the fillet. This is continued until the illuminant has reached the proper thickness, which varies with the voltage and candle-power in practical use. In any case, however, the illuminant should be made thick enough to be self-supporting, and it should be remembered that the resistance of the deposited metal must be great enough to supply the heat necessary for its own incandescence, as the fillet forms no part of the illuminant proper. The composition of the oxychlorid varies with the different metals of this group, but the reduction by hydrogen and heat is accomplished whatever this composition may be.

In the case of molybdenum I prefer to carry out this generic process in the following specific manner: The formation of the oxychlorid is carried out by treatment of molybdic acid with hydrochloric acid in the presence of heat. The reaction occurring is:  $\text{MoO}_3 + 2\text{HCl} = \text{MoCl}_2\text{O}_2\text{H}_2\text{O}$ . The temperature employed should be from 150° to 200° centigrade. This treatment results in the production of a heavy gaseous oxychlorid, which is permitted to fall upon the heated fillet, while at the same time a current of hydrogen is caused to mingle therewith. Of course the mixture of the two gases may, if desired, be accomplished before they are conducted to the fillet, but I prefer in practice the former process. It will of course be remembered that owing to the great difference in specific gravity between the oxychlorid gas and the hydrogen they will be better mingled by permitting the former to move downward in the mixing-chamber while the latter moves upward, the oxychlorid being admitted at the top of the chamber and the hydrogen at the bottom.

The fillet is heated at first to a temperature of from 800° to 1,000° centigrade, in order that the first layer of metal deposited from the mixture may be caused to adhere intimately to the surface of the fillet. The color of the fillet at this point in the process should be a cherry color of considerable brilliancy. After the deposition commences I have found it best to cause a reduction of temperature by rheostatic means, reducing the temperature as the building up of the filament takes place.

The temperature during the greater part of this treatment and after the first few moments should be about 700° centigrade, or a red heat.

The oxychlorid of molybdenum is reduced according to the following formula:  $\text{MoCl}_2\text{O}_2\text{H}_2\text{O} + 6\text{H} = 2\text{HCl} + 3\text{H}_2\text{O} + \text{Mo}$ .

The apparatus whereby this process is carried out may be of any suitable description, it being understood that proper ordinary means are employed for leading the gases to the mixing-chamber for heating the same and for carrying off the waste products as fast as deposition takes place. I do not, therefore, herein claim any particular apparatus, as those skilled in chemistry will be able to carry out this process in many well-known ways. Of course it will be understood that the fillet is preferably heated by passing an electric current therethrough, but that any other means of heating is appropriate which is consistent with the exclusion of foreign gases from the mixing-chamber and the fillet.

The particular metal employed for the illuminant is immaterial so long as one or more of its gaseous chlorin compounds, and particularly its oxychlorid, is capable of non-explosive reduction by hydrogen and heat and so long as when reduced it is refractory enough to serve for a commercial incandescent lamp.

The particular substance employed for the fillet is immaterial so long as it is capable of being formed into a fine thread-like structure and does not form a compound with the superposed illuminant.

What I claim is—

1. The method of forming illuminants for incandescent lamps which consists in imparting the desired shape to a conducting-fillet, immersing said fillet in a mixture of hydrogen and a gaseous chlorin compound of a refractory metal, and heating the fillet while so immersed, substantially as described.

2. The method of forming illuminants for incandescent lamps, which consists in imparting the desired shape to a conducting-fillet, immersing said fillet in a mixture of hydrogen and a gaseous oxychlorid of refractory metal, and heating the fillet so immersed, substantially as described.

3. The method of forming illuminants for incandescent lamps which consists in imparting the desired shape to a conducting-fillet, immersing said fillet in a mixture of hydrogen and a gaseous oxychlorid of a refractory metal, and passing an electric current through said fillet of sufficient volume to heat the same to such a temperature as to cause the deposition of the metal from the gaseous mixture, substantially as described.

4. The method of forming illuminants for incandescent lamps, which consists in imparting the desired shape to a conducting-fillet, immersing said fillet in a mixture of hydrogen and molybdenum oxychlorid, and heating the fillet so immersed, substantially as described.

5. The method of forming illuminants for

5 incandescent lamps which consists in imparting the desired shape to a conducting-fillet, passing gaseous hydrochloric acid over heated molybdic acid, mixing the gas so formed with hydrogen, heating said fillet and immersing it in the mixture while hot, substantially as described.

6. An illuminant for electric lamps composed exclusively of an incandescing body of molybdenum, substantially as described.

7. An illuminant for electric lamps com-

posed of an incandescing body of molybdenum, and containing a platinum fillet, substantially as described.

In testimony whereof I have hereunto subscribed my name this 26th day of March, A. D. 1894.

A. DE LODYGUINE.

Witnesses:

JAMES WM. SMITH,  
HAROLD S. MACKAYE.